

Sept. 27, 1938.

A. T. SHRUM

2,131,599

MANUFACTURE OF MINERAL WOOL

Filed Aug. 6, 1934

2 Sheets-Sheet 1.



INVENTOR  
*Arthur T. Shrum*  
BY  
*Henry W. Kachel*  
ATTORNEY

Sept. 27, 1938.

A. T. SHRUM

2,131,599

MANUFACTURE OF MINERAL WOOL

Filed Aug. 6, 1934

2 Sheets-Sheet 2



INVENTOR  
Arthur T. Shrum

BY  
Henry W. Kachel  
ATTORNEY

## UNITED STATES PATENT OFFICE

2,131,599

## MANUFACTURE OF MINERAL WOOL

Arthur T. Shrum, Poland, Ohio, assignor, by  
mesne assignments, to William C. Coryell,  
Youngstown, Ohio

Application August 6, 1934, Serial No. 738,619

2 Claims. (Cl. 49—77.5)

This invention relates to mineral wool, and particularly to method of and apparatus for its production.

Mineral wool is produced by directing a stream 5 of molten slag, silica rock, or earthen fines, into a violent jet of steam or air. The jet discharges into a so-called blow-room, and ordinarily the stream of slag or other suitable material is caused 10 freely to fall athwart the jet. As the steam progressively encounters the jet, the molten material 15 is progressively dispersed in the form of fine, elongated shreds or fibres. These fibres fall to the floor of the blow-room, where they form an interlaced, matted and fibrous mass which, when 20 15 the fibres cool and solidify, comprises mineral wool, or as it is commonly known, rock wool. This wool is widely used as a heat-insulating material.

In mineral wool, as it has hitherto been produced, there is found not only the desired glass-like fibres, but many small solid globules which are known as shot or beads. The shot content 25 of the wool varies, often running as high as fifty percent, by weight, and, manifestly, in proportion to the relative quantity in which the shot is present, the heat-insulating properties of the wool are impaired. This situation has proved a problem to the art, and, in seeking a solution 30 of such problem, I have made several important discoveries. I have discovered that the temperature and the analysis of the molten material, immediately prior to its introduction to the blasting jet, has a direct bearing on the quantity of shot 35 in the wool; additionally, I have found that the temperature and motion of the air in the blow-room affect the quantity of shot in the wool, as well as being partly instrumental in determining the length and physical characteristics of the fibres thereof. My invention lies in method of 40 and apparatus for readily controlling these factors, whereby I produce a wool having either no shot content or a uniform, minimum shot content,—a wool whose fibres are long and possessive of the desired high flexibility and resistance to 45 rupture.

Turning to a consideration of how the molten material is prepared for "blowing" into wool, it will be perceived that my invention embraces still other features. In passing, it may be remarked that in some cases the molten slag of a 50 blast furnace (or other metallurgical furnace) has been directly employed as the material from which to "blow" mineral wool. In general, however, it may be said that the use of "direct" slag has proved unsatisfactory, because of the un-

controllable variations in slag analysis. So far as I am aware, the best prior practice has been to melt down,—say by means of a cupola—a charge of material or materials of predetermined characteristics. The material (or materials) and coke 5 are placed in alternate layers in the cupola, until the cupola is filled, and, in accordance with usual cupola operation, air for the combustion of the coke is forced inward through tuyères located at or above the cupola hearth. Thus, the 10 massed layers of the material are melted and drawn off and "blown" into wool.

Contrary to this practice of mass melting, so to speak, I prepare the material in pulverized or comminuted condition, and progressively and 15 continuously disseminate it through a fusing atmosphere. In passing through such atmosphere the particles of material are melted or preheated, whence they are caused to enter a molten pool 20 of the material, which pool feeds a continuous stream to the wool-forming jet. The feeding of the comminuted material may be continued indefinitely, and may be effected automatically; from moment to moment the kind and quality of the material fed through the fusing or preheat- 25 atmosphere may be selected and varied, so that the analysis of the molten pool may be held to desired value; and the temperature of the fusing atmosphere may be regulated and the rate 30 of feeding of the particles may be correspondingly adjusted, whereby the temperature and volume of the molten supply pool are subject to ready control. Accordingly, it becomes possible to manufacture mineral wool in a continuous process,—a continuous process in which the critical factors alluded to above are subject to adjustment and control, readily and in a moment. I may add, my invention admits of the use of certain desirable materials and slag fines which in 35 the prior cupola practice mentioned could not be properly melted.

An object of this invention is to provide an apparatus and a method for producing mineral wool continuously which will be substantially free of shot and in cases where any shot is desired it 45 will also be possible to regulate the shot content and make it uniform throughout the production.

Another object of the invention is to provide a method and apparatus for producing mineral wool substantially uniform in quality with regard 50 to its chemical analysis, out of a slag that may be non-uniform in analysis.

A further object of the invention is to control the length of fiber of the material which is accomplished by controlling the temperature of the mol- 55

ten material and controlling the temperature of the blow-room and motion of the air currents set up in the blow-room.

Still a further object of the invention is to produce a mineral wool which will be superior in quality with regard to length and flexibility of fiber.

These and further objects will be more definitely explained and apparent from the description hereinafter contained.

In the accompanying drawings Fig. I is a view in vertical section of apparatus embodying the invention;

Fig. II is a similar view, illustrating certain modifications;

Fig. III is a view in cross-section, taken on the plane III—III of Fig. II.

Advantageously, the apparatus for the practice of my invention comprises a furnace having a tall shaft 3 extending upward from a firing chamber 30. The furnace is constructed of refractory material, reinforced and braced with steel where needed. Opening into the firing chamber 30 is a plurality of burners 10 connected to a gaseous fuel supply (not shown). Enveloping and spaced from the body of shaft 3 is a jacket 11, connected by a down-comer 11a to a manifold 12, and conduits 12a extend from the manifold and severally communicate with the openings in the furnace wall into which the burners 10 project. In service, the air for combustion of the fuel is preheated in jacket 11, and passes into manifold 12 by way of down-comer 11a, whence it is drawn through passages 12a and enters the firing chamber 30 with the jets of fuel.

Beneath the firing chamber 30 is a hearth 30a, from which a discharge passage 14 extends to a discharge mouth 16. The bottom portion 13 of the furnace, including the hearth 30a, is preferably separable from the stack portion, so that it may be independently removed for repair.

Combustion of the fuel progresses in chamber 30 and the hot waste gases flow upwardly through the shaft 3 and into a chimney 31. Adjacent the top of the shaft a cone 4 is secured, and the hot and burning gases in chamber 30 and shaft 3 are effective to provide the fusing atmosphere in which to disseminate the material, as already described. A chute 5 projects through the wall of shaft 3 and its discharge end is directed toward the cone or bell 4; a hopper 7 is maintained in supply with the comminuted material by means of an endless conveyor or elevator 8; and a vibrating feeder 6 (diagrammatically indicated, but of well-known structure) controls the progressive feeding of material from the hopper 7 to the chute 5. The chute 5 may preferably be in the form of a closed pipe forming the casing of a spiral screw conveyor which will continuously feed the material to the furnace so that it will fall upon the bell 4 and is thereby disseminated and scattered for descent through the fusing atmosphere. This pipe may be sealed against the internal pressure in the furnace when necessary to feed the furnace under pressure.

The small particles descend and float downward through the shaft against the upward, counter currents of hot gases. The velocity and temperature of these gases may be varied by regulating the quantity and pressure of air and fuel introduced into the firing chamber 30; conveniently a powerfully driven fan 32 in down-comer 11a is effective to maintain the preheated air in manifold 12 at super-atmospheric pressure, while adjustable dampers 33 in passages 12a afford a

more minute control of the air entering the combustion chamber. Manifestly, valves in the fuel supply lines may be adapted to control the pressure and quantity of fuel fed into chamber 30. Accordingly, by so varying the upward velocity 5 of gases in the shaft 3, the downward movement of the particles falling from bell 4 may be accelerated or retarded; by varying the quantity of fuel fed into the chamber 30, the temperature of the fusing atmosphere may be regulated, whereby 10 compensation is made for variations in the particle size of the material fed into the shaft, and for variations in the rate of feeding, so that upon reaching the bottom of the chamber 30, the particles may be completely fused and form a molten 15 pool on the hearth 30a.

In the practice of my invention the accessibility of each particle (and of the whole surface area of each particle) to the hot gases renders it possible to fuse certain materials which otherwise 20 could not be properly fused. Thus, greater varieties of material may be used, and the field from which the raw material is obtained is appreciably widened.

While many of the falling particles will actually 25 melt during falling some of them may reach the bath in a solid condition due to the difference in size of the particles. Those that are melted will tend to superheat and then the molten bath will equalize the temperature of the particles so that 30 all of them will eventually be melted.

It may be remarked that the height of the stack may be designed to meet particular conditions in the field. That is to say, if certain material is difficult to fuse, other things being equal 35 a higher stack will be used; if the material is readily fusible, a lower stack may be used. In actual tests I have found that blast furnace slag of 60 mesh particle size was well fused in a stack 20 feet high, and it appeared that good results are 40 obtainable with particle sizes of from 40 to 100 mesh and a heating zone temperature of about 2700° F.

The feeding of material into the shaft 3 is so determined that a pool of relatively large volume is maintained on the hearth 30a, in which the temperature of varying sized particles become 45 equalized. The viscosity and temperature of the molten material in the pool are maintained as desired, by regulating the rate of combustion 50 in chamber 30. A continuous stream of molten material flows through passage 14, and falls from mouth 16 into a jet of steam delivered by pipe 17. This steam may be super-heated, the excess 55 temperature being obtained by super-heating the steam in the furnace stack or in any other suitable manner. As already mentioned, the jet of steam (or other suitable fluid) "blows" the material into tails of fibres glasslike. In accordance 60 with known practice, a small quantity of oil may be introduced to steam line 17, to produce a more fluffy, flexible product. The jet is directed through an opening 23 in the wall 19 of blow-room 18, and as already mentioned the 65 fibres fall to the floor of the blow-room and form a "blanket" of mineral wool thereon. The blow-room is an elongate room, a room of such dimensions that it is impossible for the molten slag to make contact with its walls before the 70 fibers have been fully formed. As usual, the floor of the blow-room comprises the upper reach of an endless conveyor 20 for removing the wool, and by regulating the speed of the conveyor, it is possible to vary the thickness of said blanket. 75

and at the time interval during which the fibres remain in the blow-room.

In the operation of the furnace there is a tendency for cold air to filtrate into the passage 14 and to destroy the precisely determined temperature of the molten material on its way to the steam jet unless this passage is full of molten material. I have found that this objectionable condition may be remedied by providing a burner 15, to direct burning fuel into the passage 14 adjacent its mouth 16, so that a slight pressure will be formed at the mouth.

During the continuous wool-blowing operation, the hot steam jet aspirates cold air from the outer atmosphere inward, through the opening 23. The foregoing specification has mentioned how the temperature and air currents in the blow room have a very definite effect upon the physical characteristics of the fibres and upon the quantity of shot produced in the wool. In accordance with the invention, I stabilize and regulate atmospheric conditions within the blow-room. The quantity of heat entering the blow-room is supplied by the steam jet and the molten slag, and in my continuous process this heat supply, together with the chilling effect of the cold air entering opening 23, is of relatively constant value. Advantageously, I provide one or more vents 22 in the walls of the blow-room, say in the top wall 21; the vent area is adapted to be varied by gates 24 subject to the control of a line 25, whereby the escape of air, vapors, and dust from the blow-room may be established and maintained at constant rate. Thus in regulating the escape of the air and vapors from the blow-room, the quantity of cold air entering opening 23 is regulated, and in consequence the atmospheric conditions within the blow-room are subject to the hand of the operator. Indeed, well-known thermostatic instrumentalities may be organized to shift the wire 25 automatically, or in other convenient manner may be adapted automatically to regulate the blow-room atmosphere.

In proceeding in accordance with this invention, I am able to produce a wool of superior character,—a wool whose fibres are long and flexible, and a wool having a shot content below 10 percent by weight.

It has always been realized that many advantages and economies might be effected, if molten slag direct from a blast furnace were used as the material of which to produce the wool, but as above remarked it has hitherto been impractical to use "direct" slag, because of the variations in the analysis thereof. In providing for a continuous or progressive melting or suitable material, as above described, it is possible from moment to moment to alter the material being fused, whereby it becomes feasible to use "direct" slag, as will be understood upon referring to the modification illustrated in Figures II and III.

The modified apparatus embodies the shaft 3 and feeding mechanism (4 to 8) described in Figure I. The hearth 30b of the modified furnace is relatively large and is adapted to hold a large store 28 of slag, delivered from a so-called thimble 27 and entering the furnace through an inlet 26. The thimble is the usual type of railway vehicle used to transport molten slag from a blast furnace to a dump or other place of disposal.

Burners 10 (Fig. II) are inserted above the

hearth 30b, and serve to create the fusing atmosphere in the stack 3. It will not always be necessary under all conditions to use the burners 10 as electrodes will furnish heat to the bath material and convection will cause warm air currents to move up the furnace stack. When these air currents are sufficiently hot it will then not be necessary to use the burners 10 in this type of furnace. The material fed into the stack 3 is of such chemical composition as to bring the pool 28 to desired analysis, and thus the blast furnace slag is rectified for conversion to mineral wool. I contemplate that electric current may also be employed to keep the pool 28 at proper temperature, and to this end I show in exemplary way a plurality of electrodes 29 projecting into the pool. The position of the electrodes in the pool may be adjusted by a gear-and-ratchet mechanism 130 and slag-heating electric currents are caused to flow in the pool from one electrode to another.

The molten material passes from the hearth 30b by way of passage 14, and is blown into wool in the manner already described.

I have used the word "continuous" in this specification and in the claims to mean that material can be fed into the furnace melted and run out continuously to distinguish it from the process of charging a furnace similar to a cupola with a certain definite charge and melting it down to produce a given quantity of molten material. In my invention it is possible to continuously feed and melt and run the material out without depending upon a single charge and a single melting period.

While I have shown and described the preferred embodiment of my invention, it is to be understood that various changes in the apparatus and method may be made without departing from the spirit of the invention or the scope of my broader claims.

Having thus clearly described my invention, what I claim and desire to protect by Letters Patent is:

1. The method of making mineral wool which comprises, continuously feeding particles of a mass of comminuted fine mineral material of a size between 40 and 100 mesh in a region of heated and upwardly flowing gases whereby the material is pre-heated, progressing the particles in a freely falling manner and at a determined rate through the heating region for a sufficient length of time to melt the heated particles, collecting the molten material in a pool, discharging the molten material from the pool, and thereafter blowing the discharged molten material to break it down into a fibrous condition.

2. The method of making mineral wool which comprises, forming a pool of molten mineral material, adding molten mineral material to said pool in bulk, feeding particles of a mass of comminuted fine mineral material of selected composition and of a size between 40 and 100 mesh in a region of heated and upwardly flowing gases whereby the particles are pre-heated, progressing the particles in a freely falling manner and a determined rate through the heating region for a sufficient length of time to melt the heated particles, collecting the melted particles in the pool, discharging the molten material from the pool, and thereafter blowing the discharged molten material to break it down into a fibrous condition.

ARTHUR T. SHRUM.